

## UNITED STATES PATENT OFFICE

2,270,658

## TREATMENT OF TEXTILE MATERIALS

Wolfgang Linnhoff, Berlin-Lankwitz, Germany,  
assignor to North American Rayon Corporation,  
New York, N. Y., a corporation of Delaware

No Drawing. Application November 15, 1938,  
Serial No. 240,573. In Germany November 15,  
1937

6 Claims. (Cl. 8—120)

My present invention has to do with a new and novel process for use in the treatment of artificial silk, wool, cotton, casein and the like, and of woven and knitted fabrics made therefrom, and has to do more specifically with the chemical treatment of such fibers and the goods made therefrom in order to make them more water-repellent.

One object of my present invention is to provide a process of the type described in which the use of abnormally low temperatures, and the subsequent increase in cost of production is eliminated in this type of yarn and fabric treatment.

Another object of my present invention is to provide a new and novel treating means which gives more advantageous results than have hitherto been considered possible.

These and other objects of my invention will in part be apparent and in part pointed out by a careful consideration of the following specification and claims.

The prior art describes processes whereby products made from cellulose and cellulose derivatives, such as artificial silk, staple fibres, artificial horse-hair, and films, and also natural fibres, such as cotton, flax and even wool may be superficially esterified. It is also well known, in treatments of this type, that long chain aliphatic compounds may be employed in order to give water-repellent properties to the treated goods. Hitherto, use has been made of chlorides, anhydrides and amides of fatty acids and long chain aldehydes and isocyanates. In processes of this class it is necessary that during the esterification long chain molecules, e. g., of the paraffins become anchored on and in the cellulose fiber with the aid of appropriate reactive groups. This process, in the light of present knowledge, may be accomplished, depending upon the means of esterification, through the use of an organic non-solvent of cellulose, such as benzene, carbon tetrachloride and the like. A series of fatty compounds, for example, esterifying agents, such as anhydrides, amides, aldehydes and the like, emulsified in water, may also be used.

It has been found that when water has been used in the prior art as a medium certain esterifying agents, such as anhydrides, become ineffective because they saponify prematurely. In practice it has been found that many inconveniences arise because of this saponification. Hitherto this emulsion has been made, for example, from fatty acid anhydrides using the common admixtures of soap and sodium carbonate. A considerable saponification has been found to

occur during and shortly after the production of the emulsion even when there was a strict temperature control maintained. In large scale production it has oftentimes been impossible to immediately use the prepared compounds and as a result extensive saponification continuously occurs. It is necessary to dry and harden fibres which have been treated with this preparation. By reason of this there is also danger that, when water and heat are employed, a further portion of the reagent employed becomes saponified and therefore valueless from an industrial standpoint. Therefore, it has become common in the industry to dry the impregnated product through the use of low temperatures over a considerable period of time, thus materially increasing production costs. Despite precautions of this type, however, it has been found that a large portion of the anhydride becomes saponified and thus lost. This means that a large percentage of the reagent is unable to perform its normal function in the reaction and, as a result, the water-repellent effect on the fibre either does not occur or, if it does, occurs only to a limited extent.

I have now found, and this is the basis of my present invention, that it is possible to produce emulsions from fatty acid anhydrides and the like which are much less subject to saponification and which at the same time exert no destructive influence upon the products treated, for example, fibres. Tests have shown that certain organic materials in the form of quaternary nitrogen compounds can produce emulsions of fatty acid anhydride, for example, of the class of stearic acid anhydride, or anhydrides such as are obtained from hardened train oil (blubber), etc., in water. In the emulsions thus obtained, only a very small saponification takes place in the aqueous medium as well as on the fibre. Water-soluble quaternary nitrogen compounds of paraffins with at least 10 carbon atoms have proved to be appropriate emulsifying agents which are, for example, of the



and in which R represents the paraffin chain, and where other halides may be substituted for chlorine.

50 I have also found that, among others, lauryl-pyridine chloride, cetyl-pyridine chloride, cetyl-pyridine bromide, cetyl-pyridine iodide as well as stearyl-pyridine chloride are valuable as emulsifying agents.

55 The use of acid anhydrides of hardened train

oil (blubber) and a mixture of cetyl-pyridine chloride and stearyl-pyridine chloride, such as may be obtained from technical stearin, has also produced very favorable results. High molecular pyridinium halides, obtained from hardened train oil (blubber), may also be used.

In order to more definitely indicate the manner in which my present invention may be used in the industry, I shall give three examples which will serve to clearly point out several possible uses.

*Example I*

5 kg. of a mixture of cetyl-pyridine chloride and a stearyl-pyridine chloride, such as are obtained from stearin, are dissolved in 500 liters of softened water and heated to 70° C. Then 20 kg. of acid anhydrides derived from train oil (blubber) are melted and introduced with stirring, in a thin jet, into the aqueous solution. Subsequently the entire mass is diluted with another 500 liters of cold water, stirred and then further cooled. The fine emulsion is now ready for use and 40 kg. of staple fibres are added to the emulsion and the fibre mass is well soaked therein. After treatment in the emulsion, the staple fibres are thoroughly hydro-extracted in a centrifuge and placed in loose layers on a belt drier and dried at a temperature not exceeding 50° C. As soon as the water is extracted, the drying temperature is increased to approximately 100° C. and maintained there until the water-repellent effect becomes fast enough so that it will resist boiling. This usually requires approximately one hour.

*Example II*

The same procedure as outlined in Example I is followed, with the exception that a mixture of cetyl pyridine bromide and stearyl pyridine bromide is used. This mixture is known in the industry under the trade name "Fixanol."

*Example III*

The same procedure as outlined in Example I is followed, with the exception that lauryl pyridinium chloride is used as emulsifying agent, together with ordinary well water and that the drying is carried out at 70° C.

Instead of staple fibres, other textile materials, such as artificial silk, cotton, flax, wool, casein fibres, also in the form of fabrics and woven material, as well as artificial horse hair and films may be treated in a similar way.

Modifications of my invention will readily be recognized by those skilled in the art, and I desire to include all such modifications coming within the scope of the appended claims. In these claims the term "water-soluble cation-active compounds" includes cation-active compounds which are sufficiently water-soluble to furnish surface-active cations therein, and the term "textile material" embraces filaments, fibres, threads, etc., as well as fabrics, knitted or woven cloths, films etc., of natural or synthetic fibres.

I claim:

1. In the process of rendering textile materials water repellent, the steps which comprise treating a textile material with an emulsion comprising a substantially water insoluble, long chain, aliphatic anhydride esterifying agent, a water soluble cation-active quaternary ammonium compound having an aliphatic radical of at least 10 carbon atoms, and subsequently heating said treated material to cause esterification

thereof, said cation-active compound present in said emulsion acting to substantially reduce saponification of said esterifying agent in said water.

5. In the process of rendering textile materials water repellent, the steps which comprise treating a textile material with an emulsion comprising a substantially water insoluble, long chain, aliphatic anhydride esterifying agent, a water soluble cation-active pyridinium compound having an aliphatic radical of at least 10 carbon atoms and water, and subsequently heating said treated material to cause esterification thereof, said cation-active compound present in said emulsion acting to substantially reduce saponification of said esterifying agent in said water.

3. In the process of rendering textile materials water repellent, the steps which comprise treating a textile material with an emulsion comprising a substantially water insoluble, long chain, aliphatic anhydride esterifying agent, water and a water soluble cation-active pyridinium halide having the structure

25 R—N—halogen



30 in which R represents a hydrocarbon chain having at least 10 carbon atoms derived from hardened blubber, and subsequently heating said treated material to cause esterification thereof, said cation-active pyridinium halide present in said emulsion acting to substantially reduce saponification of said esterifying agent in said water.

4. In the process of rendering textile materials water repellent, the steps which comprise treating a textile material with an emulsion comprising a substantially insoluble, long chain, aliphatic anhydride esterifying agent, lauryl pyridinium chloride and water, and subsequently heating said treated material to cause esterification thereof, said lauryl pyridinium chloride present in said emulsion acting to substantially reduce saponification of said esterifying agent in said water.

5. In the process of rendering textile materials water repellent, the steps which comprise treating a cellulosic textile material with an emulsion comprising a substantially water insoluble, long chain, aliphatic anhydride esterifying agent, a water soluble cation-active quaternary ammonium compound and water, and subsequently heating said treated material to cause esterification thereof, said cation-active compound present in said emulsion acting to substantially reduce saponification of said esterifying agent in said water.

6. In the process of rendering textile materials water repellent, the steps which comprise treating a cellulosic textile material with an emulsion comprising a substantially water insoluble, long chain, aliphatic anhydride esterifying agent, a water soluble cation-active pyridinium compound and water, and subsequently heating said treated material to cause esterification thereof, said cation-active compound present in said emulsion acting to substantially reduce saponification of said esterifying agent in said water.

WOLFGANG LINNHOFF.